

## 1

3744,971

**FUEL-METAL COMPATIBILITY TEST UNIT**  
Vernon A. Lamb, Royal, Iowa, Wahling H. Ng, Rockaway, N.J., and John P. Young, Gaithersburg, Md., assignors to the United States of America as represented by the Secretary of the Army

Filed May 28, 1971, Ser. No. 148,063

Int. Cl. G01n 31/10, 33/22

U.S. Cl. 23—230 R

7 Claims

### ABSTRACT OF THE DISCLOSURE

A method and test apparatus is presented which measures gas produced by catalytic decomposition or chemical reaction of a hydrazine-type fuel and a metal specimen.

The invention described herein may be manufactured, used and licensed by or for the Government for governmental purposes without the payment to us of any royalties thereon.

The development of high strength/low weight materials, such as nickel maraging steel, cryogenically formed stainless steel, and titanium alloys have provided designers with structural materials possessing yield strengths of up to 400,000 p.s.i. Fabrication of tankage from these materials results in higher ratios of payload to total weight of missile (or a greater range and shorter time-to-target) which is the goal of rocket technology.

A lack of compatibility, however, of some of these materials with certain liquid propellants has restricted their use as tankage. One corrective approach has been to provide an internal metallic protective coating which neither reacts with nor catalyzes a decomposition of the particular liquid propellant. Such a coated material may be said to be compatible with the propellant if it fulfills the above requirements. Since a five year storage life is desired in prepackaged liquid rockets, it is clear that a method and apparatus to predict long term gaseous buildup from propellant decomposition-reaction is needed. Such exposure tests must be at least of one year duration and at an elevated temperature (to accelerate any chemical or catalytic reactions) to be meaningful.

It is therefore an object of this invention to provide a method of determining gaseous buildup from liquid propellants induced either catalytically or through chemical reaction with a high strength material tankage.

Yet another object of this invention is to provide an apparatus to measure the above mentioned gaseous buildup.

A still further object of this invention is to provide an apparatus superior to previous units in the quantitative containment of the gaseous vapors released by the propellant fuel.

Other objects and many of the attendant advantages of this invention will be readily appreciated as the same become better understood by reference to the following description.

This invention relates to a method of determining the rate of decomposition of a liquid fuel, preferably a hydrazine-type fuel, and presents an apparatus for the quantitative measurement of gases evolved from the fuel caused by catalytic decomposition or reaction with high strength-low weight metals used as tankage with said fuels.

## 2

### DESCRIPTION OF THE APPARATUS

A preferred embodiment of the apparatus consists of a heat resistant glass unit incorporating a chamber 1 for holding the fuel 2, for example a hydrazine-type fuel and metal specimen 3 and an attached calibrated (centimeter scale) mercury-filled manometer 4 to measure any gas released by catalytic decomposition or by reaction of the specimen whose compatibility with the preferred hydrazine fuel is being tested. The various legs of the manometer and fuel test bulb are strengthened with glass braces 5. An enlarged section of the manometer near the fuel bulb allows for a reservoir of mercury to increase the time interval between adjustments of the level of mercury in the manometer due to release of gas by any reaction during the test and also permits use of a shallow temperature bath (necessary to accelerate decomposition or reaction in simulated storage testing) by reducing the length of the manometer section of the unit.

Initially the ends of the specimen chamber are left open to load the specimen and the fuel and then are fusion-sealed to contain the gas vapors. All areas of the unit contacted by the fuel or fuel vapors are arranged to be below the surface of the constant temperature bath to reduce transfer of the fuel to the manometer side of the unit by condensation.

A porous frit 6 with holes too small to permit the passage of mercury between the test chamber and the manometer is installed in a connecting tube 7 which is sloped toward the test chamber to return any fuel condensate to the chamber. The apparatus has a centimeter scale attached to the manometer tube which allows reading of the height of the mercury column indicating changes in the pressure and volume of the gas evolved from the propellant.

Such a fusion closed system, as above, was arrived at when it was found that closure seals (a stop cock type system) employing closure greases such as, vaseline, silicone grease, vacuum pump oil or Teflon (tetrafluoroethylene) grease, were inadequate. Leakage problems were encountered due to the greases' solubility and reactivity with the hydrazine fuel vapors and secondly the high temperature (160° F.) at which the experiment was carried out.

### DESCRIPTION OF THE TEST METHOD

The glass apparatus was checked with a preloading leak-test procedure which consisted of two tests.

The unit was cleaned by the following steps: (a) Submerge and soak in a nitric acid solution (1:1 dilution of conc.  $\text{HNO}_3$ ) for two hours. (b) Rinse with distilled water. (c) Soak two hours in aqueous  $\text{NH}_3$  (1 part conc.  $\text{NH}_3$  plus 4 parts  $\text{H}_2\text{O}$ ). (d) Rinse with distilled water. (e) Oven dry.

The unit was then clamped in an inverted position. The specimen to be tested (previously cleaned by conventional pre-plating procedures, followed by a soak in the above  $\text{NH}_3$  solution, rinsed, and air-dried) was inserted into the specimen chamber through its open end. The specimen chamber was then sealed by fusing and drawing the glass. Adequate precautions were taken during this operation to avoid heating and oxidizing the specimen (step-wise drawing with intermittent cooling, air blast cooling of the outside of the opposite end of the specimen chamber, and simultaneous flushing of the specimen chamber with nitrogen). The unit was then pumped down to a

low pressure through the open end of the manometer tube and all seals were checked with a spark-type, high voltage leak tester. Leaks, if found, were repaired. For further leak-testing, mercury was then added to the manometer and the unit was pressurized with  $N_2$ , using a 2 mm. Teflon tube pushed through the mercury column, to the limit of the manometer tube, thus exposing all fusion seals and joints to the gas.

After about two weeks, if no evidence of a leak was observed, the units were then opened by breaking the seal at the top of the specimen chamber and enough fuel was added to cover the specimen.

A plastic syringe with its needle attached to a 2 mm.-dia. Teflon tube was used to introduce the fuel into the lower end of the specimen bulb without wetting the wall of the inlet tube. A temporary closure of the inlet tube was then made with a Teflon plug. The fuel was left in the unit about one week to leach possible residual impurities from the specimen and the interior of the unit. This fuel was then removed by use of the syringe and replaced with fresh fuel, again avoiding wetting of the upper end of the inlet tube. If wetted at this point, it was sometimes difficult subsequently to obtain a leak-free fusion seal.

The fuel inlet at the top of the specimen chamber was then resealed by fusion. The seal was inspected under magnification. If perfect, the unit was flushed (alternately pressurized and depressurized) with  $N_2$  by inserting a long, 2 mm.-dia. Teflon tube through the open end of the manometer, through the mercury, and into the gas chamber above the mercury in the manometer bulb. The unit was then placed in the constant temperature bath to begin the test.

One specimen chosen was coated 18% nickel maraging steels (18-18.5% nickel, 2-4.8% molybdenum, 0.2-0.65% titanium, 0.1% aluminum, 0.03% maximum carbon, 7.8-8.7% cobalt, balance iron). Particular coatings included aluminum, cadmium, nickel, 50/50 lead-tin solder, silver, chromium, gold, tin, zinc and cobalt.

Other specimens tested were molybdenum metal (99.9% molybdenum); cryogenically formed stainless steel 301 (17% chromium, 7% nickel, 0.15% maximum carbon, balance iron); AM 355 (15.5% chromium, 4.5% nickel, 3% molybdenum, balance iron); Inconel 718 (18.6% chromium, 18.5% iron, 0.4% aluminum, 0.9% titanium, 3.1% molybdenum, 0.04% carbon, 5% columbium, balance nickel); and Ti-6Al-4V (6.5% aluminum, 4% vanadium, 0.08% maximum carbon, 0.25% maximum iron, 0.05% nitrogen, 0.015% maximum hydrogen, balance titanium).

Fuels tested include hydrazine, monomethyl-hydrazine, unsymmetrical dimethyl hydrazine and mixtures of the above.

After approximately one year the change in volume and pressure due to gas evolved by decomposition of the propellant was measured and the following calculations made to determine the decomposition rate of the particular specimen-fuel system.

The equation:

$$\Delta V_{t,a} = \frac{V_2 P_2 - V_1 P_1}{P_a} \quad (1)$$

gives the amount of gas evolved, measured at atmospheric pressure ( $P_a$ ) where  $V_1$ ,  $V_2$  and  $P_1$ ,  $P_2$  are initial and final total volume and pressure respectively in the apparatus. The volume of the zero point of the manometer is determined from initial calibration of the apparatus. From this value and the measured shift of the manometer level,  $V_1$  and  $V_2$  are calculated. Height of the mercury in the manometer plus atmospheric pressure yield values of  $P_1$  and  $P_2$ . The amount of gas evolved as calculated from

Equation 1 is due in part to catalytic decomposition at the surface of the metallic specimen, and in part from the inherent tendency of the propellant to decompose at other locations, e.g., in the liquid itself, in the vapor phase, and at the glass propellant interface. The latter, referred to as "background decomposition," is determined in an identical apparatus, except that no specimen was present, and is subtracted from the volume of Equation 1 to obtain the actual amount of gas evolved due to the specimen.

Since the catalytic decomposition rate of gas evolved due to contact of a given specimen with the propellant is proportional to the area of the specimen and to the time of contact, the reactivity might be expressed in terms of a single coefficient defined as rate of gas evolved per unit area per unit time.

As per Equation 1,  $\Delta V_{t,a}$  is the total volume of gas evolved, measured at 1 atmosphere pressure, that would change the volume and pressure in the system from  $V_1$  and  $P_1$  to  $V_2$ ,  $P_2$ . If  $\Delta V_{b,a}$  is the volume similarly determined due to background condition, and  $d_t$ ,  $d_b$  are respective days of test, and  $A_s$  is the area of the specimen, then  $R_s$ , the rate coefficient, would be as follows:

$$R_s = \frac{\Delta V_{t,a}/d_t - \Delta V_{b,a}/d_b}{A_s} \quad (2)$$

$R_s$  is expressed as  $\text{cm}^3/\text{day}/\text{cm}^2$ .

For convenience, the rate of decomposition is also expressed in terms of specimen-tank pressure after one year, assuming a one cubic foot tank with 10% ullage, and with the entire inner surface active. Pressure in this assumed tank would be proportional to the rate coefficient. The relationships are indicated as follows:

$V_u$  = ullage volume = 10% of 1 ft.<sup>3</sup> = 2,832 cm.<sup>3</sup>  
 $\Delta V_y$  = volume of gas evolved in 1 year in cm.<sup>3</sup>, measured at 1 atm., also

$\Delta V_y = (R_s) (d_t) (A_s)$   
 $= (R_s) (365 \text{ days}) (5,574 \text{ cm}^2)$   
 $P_a$  = standard atmospheric pressure, 14.7 p.s.i.  
 $P_y$  = pressure developed in tank after 1 year, p.s.i.

Applying the gas law and treating the specimen-tank as a closed system (fixed volume), the following equation can be obtained.

$$P_a(V_u + \Delta V_y) = P_y V_u \quad (3)$$

solving (3) for  $P_y$ :

$$P_y = P_a + \frac{\Delta V_y P_a}{V_u}$$

$$= 14.7 \text{ p.s.i.} + \frac{(R_s) (365) (5,574) (14.7)}{2,832}$$

$$= 14.7 \text{ p.s.i.} + 10,560 R_s \quad (4)$$

In Equation 4  $P_y$  is absolute pressure. If  $P_{y,g}$  is designated as gage pressure (p.s.i.g.) after one year, then

$$P_{y,g} = 10,560 R_s \quad (5)$$

The above equations are derived directly from the simple gas law. Corrections might have to be applied for errors due to gas law deviations, change of ullage owing to expansion of liquid propellant with increase of temperature, etc., if such errors are significant in a given system.

The following represents test data for specimens exposed to MHF-3<sup>a</sup> at 160° F. for various periods of time obtained by using the apparatus and method disclosed herein.

<sup>a</sup> A mixture of hydrazine and monomethyl hydrazine.

| Specimen                                  | Area of specimen (cm. <sup>2</sup> ) | Time under test (days) | Gas evolved <sup>b</sup> (cm. <sup>3</sup> ) | Rate coefficient (cm. <sup>3</sup> /day/cm. <sup>2</sup> ) | Calculated tank pressure after one year <sup>c</sup> (p.s.i.g.) |                                                                 |
|-------------------------------------------|--------------------------------------|------------------------|----------------------------------------------|------------------------------------------------------------|-----------------------------------------------------------------|-----------------------------------------------------------------|
|                                           |                                      |                        |                                              |                                                            | Rate coefficient (cm. <sup>3</sup> /day/cm. <sup>2</sup> )      | Calculated tank pressure after one year <sup>c</sup> (p.s.i.g.) |
| Aluminum <sup>a</sup>                     | 12.5                                 | 475                    | 1.1                                          | 0.00019                                                    | 2                                                               |                                                                 |
| Cadmium (thin)                            | 10.6                                 | 629                    | 6.1                                          | 0.0009                                                     | 10                                                              |                                                                 |
| Cadmium                                   | 14.7                                 | 614                    | 1.1                                          | 0.0012                                                     | 1                                                               |                                                                 |
| Cadmium (0.1 mil)                         | 14.4                                 | 27                     | 2.3                                          | 0.0059                                                     | 62                                                              |                                                                 |
| Electroless nickel                        | 22.2                                 | 788                    | 17.0                                         | 0.00097                                                    | 10                                                              |                                                                 |
| Electroless nickel (Alk-bath)             | 13.0                                 | 320                    | 42.5                                         | 0.0125                                                     | 132                                                             |                                                                 |
| Electroless nickel (BH <sub>4</sub> bath) | 14.2                                 | 390                    | 113.0                                        | 0.0203                                                     | 214                                                             |                                                                 |
| Electroless nickel (0.1 mil)              | 15.3                                 | 63                     | 7.5                                          | 0.0078                                                     | 82                                                              |                                                                 |
| Electroless nickel (heated at 800° C.)    | 12.2                                 | 305                    | 4.1                                          | 0.0011                                                     | 12                                                              |                                                                 |
| Electroless nickel (oxidized)             | 14.4                                 | 40                     | 3.5                                          | 0.0061                                                     | 64                                                              |                                                                 |
| Electroplated nickel                      | 14.0                                 | 211                    | 19.8                                         | 0.0067                                                     | 71                                                              |                                                                 |
| Silver                                    | 14.5                                 | 626                    | 2.3                                          | 0.00025                                                    | 3                                                               |                                                                 |
| Silver (thin)                             | 16.0                                 | 709                    | 128.0                                        | 0.012                                                      | 119                                                             |                                                                 |
| Solder (Pb-Sn, 50-50) (dip coated)        | 14.3                                 | 19                     | 0.4                                          | 0.0015                                                     | 16                                                              |                                                                 |
| Solder (Pb-Sn, 50-50) <sup>a</sup>        | 15.3                                 | 614                    | 0                                            | 0                                                          | 0                                                               |                                                                 |
| Tin                                       | 13.0                                 | 616                    | 26.3                                         | 0.0033                                                     | 35                                                              |                                                                 |
| Chromium                                  | 17.0                                 | 482                    | 113                                          | 0.0201                                                     | 213                                                             |                                                                 |
| Gold                                      | 22.9                                 | 222                    | 49.0                                         | 0.0095                                                     | 94                                                              |                                                                 |
| Tungsten                                  | 24.8                                 | 358                    | 46.0                                         | 0.0051                                                     | 54                                                              |                                                                 |
| Zinc                                      | 15.6                                 | 341                    | 15.4                                         | 0.0029                                                     | 31                                                              |                                                                 |
| Cobalt                                    | 16.1                                 | 199                    | -----                                        | 0.94                                                       | 9,900                                                           |                                                                 |
| Tin-nickel alloy (65-35)                  | 24.0                                 | 358                    | 51                                           | 0.0060                                                     | 63                                                              |                                                                 |
| Molybdenum <sup>a</sup>                   | 4.8                                  | 368                    | 217                                          | 0.123                                                      | 1,300                                                           |                                                                 |
| 18% Maraging Steel <sup>a</sup>           | 17.0                                 | 371                    | 485                                          | 0.097                                                      | 1,030                                                           |                                                                 |

<sup>a</sup> These specimens are solid metals. All others are coatings on 18% Maraging Steel.

<sup>b</sup> Cumulative total, corrected for background rate and to 1 atm. pressure.

<sup>c</sup> Based on a tank in the form of a cube, 1 ft.<sup>3</sup> volume, 10% ullage.

Thusly through the practice of this invention, raw data may be obtained which may be easily refined, by the provided mathematical calculation, into both rate coefficients and projected tank pressures for particular fuel-metal tankage systems.

It can be seen that the above described test device provides particular advantage in the ready accessibility provided to the test sample. The metal specimen 3 for example, may be removed from the test chamber 1 at the completion of or during the test period. A full scale field test of metal-fuel compatibility requires relatively complicated removal and sectioning of the tankage material. Such sectioning is, of course, time consuming and expensive and also requires a termination of the testing of that particular tankage-fuel system whereas the test samples when practiced with the present invention may be reinserted and further testing continued after preliminary examinations have been made.

Further, because the system is fusion sealed, inaccuracies due to leakage inherent in previous systems employing stopcocks and glass taper joints are avoided.

We wish it to be understood that we do not desire to be limited to the exact details and compositions described in this specification for obvious modification will occur to a person skilled in the art.

We claim:

1. A method for determining the rate of catalytic decomposition and chemical reaction of a liquid hydrazine fuel in contact with a metal specimen comprising the steps of:

contacting the metal specimen with the hydrazine fuel in a fusion sealed glass system consisting essentially of a glass chamber connected to a mercury manometer;

purging said system with an inert gas to displace the air and provide an inert atmosphere therein; measuring the change in pressure and volume caused by the evolution of gases from the catalytic decomposition and chemical reaction of the hydrazine fuel and metal specimen and the time period of such gas evolution;

calculating by use of simple gas laws the amount of gas evolved from the above decomposition and reaction;

deducting any inherent catalytic decomposition of the

fuel in the absence of the metal specimen; calculating the decomposition rate of the fuel expressed as cm.<sup>3</sup> of gas/cm.<sup>2</sup> area of metal specimen/day.

2. The method of claim 1 wherein the test method is carried out at an elevated temperature.

3. The method of claim 1 wherein the fuel is selected from the group consisting of hydrazine, monomethyl hydrazine, unsymmetrical dimethyl hydrazine, and mixtures thereof.

4. The method of claim 1 wherein the metal specimen is chosen from the group consisting of aluminum, 18% nickel maraging steel, molybdenum metal, cryogenically formed stainless steel, and coated 18% nickel maraging steels.

5. The method of claim 4, wherein the metal specimen is coated 18% nickel maraging steel coated with a metal selected from the group consisting of cadmium, electroless nickel, aluminum, 50/50 lead-tin solder, silver, chromium, gold, tin, zinc and cobalt.

6. An apparatus for measuring gases produced by the catalytic and chemical reaction of hydrazine-type fuels and metals comprising:

a fusion sealed glass system consisting essentially of a glass test chamber having an aperture therein for the escape of gases evolved; a mercury filled calibrated glass manometer, open to the atmosphere, connected to said aperture; and

a gas permeable partitioning means located between the test chamber and the glass manometer.

7. The apparatus in claim 6 wherein the gas permeable partitioning means is a glass frit.

#### References Cited

#### UNITED STATES PATENTS

65 1,046,259 12/1912 Bunzel ----- 23—253 R  
3,323,872 6/1967 Scott ----- 23—256 X

#### OTHER REFERENCES

70 L. F. Audrieth: The Chemistry of Hydrazine, page 102 (1951).

JOSEPH SCOVRONEK, Primary Examiner

U.S. Cl. X.R.

75 23—253 R; 149—36